

Jan. 10, 1928.

C. S. JOHNSON

1,656,001

PROCESS OF PROPORTIONING SAND AND WATER FOR CONCRETE

Filed April 19, 1926



Inventor:  
Charles S. Johnson  
By Chiridahh Parker Kalon

Attest:

## UNITED STATES PATENT OFFICE.

CHARLES S. JOHNSON, OF CHAMPAIGN, ILLINOIS.

## PROCESS OF PROPORTIONING SAND AND WATER FOR CONCRETE.

Application filed April 19, 1926. Serial No. 103,183.

- The invention relates generally to the art of making concrete and more particularly to a method for proportioning the total amount of water in the mix.
- 5 It is the object of the invention to provide a new and improved process for proportioning the total amount of water in a concrete mix, that will compensate for the normal moisture content of the sand.
- 10 It is another object of the invention to provide an improved process for proportioning the total water in a concrete mix which is readily adapted to field work.
- 15 It has been recognized that the strength of concrete depends largely upon the total amount of water in the mix, and it follows that accurate control of the total water included in the mix is highly essential to obtain concrete of uniform strength.
- 20 The methods heretofore used for proportioning the water in the mix have not given uniform results. In the processes used heretofore wherein the sand is measured by volume and then introduced into a concrete mix
- 25 with a separately proportioned unit of water, variations in the normal moisture content of the sand have caused variations in the total water in the mix. Attempts have been made to control accurately the
- 30 amount of water introduced into the mix but no process has been advanced whereby the total water could be controlled satisfactorily without adjustment to compensate for unapparent variations in the compaction of the sand.
- 35 Changes in the moisture content in commercial sand alter the apparent volume of the sand due to the resulting changes in bulking, but do not alter the absolute volume of the sand. The changes in apparent volume are not directly proportional to the changes in normal moisture content throughout the full range of possible moisture content in the sand. However, an analysis of the bulking characteristics of commercial sand has disclosed that the absolute volume of sand in equal apparent volumes of moist sand is quite constant within a certain range of moisture variation, and
- 45 records disclose that in commercial sand the normal moisture content holds quite closely within the limits of this range.
- 50 Thus the variation in absolute volume of sand measured by apparent volume is practically negligible in commercial work, and sand measured by apparent volume will give practically uniform absolute volumes independent of the normal moisture content within this range.
- 55 I utilize these facts in providing a process for proportioning the total amount of water for a concrete mix, the process consisting generally of measuring a predetermined volume of normally moist commercial sand and then combining with that sand a quantity of water such that the combined sand and total water equals a predetermined volume.
- 60 For the purpose of illustrating more clearly the operation of the process I have illustrated in the accompanying drawings an apparatus adapted to utilize the process, together with diagrammatic sectional views of the apparatus at various stages in the process. It is to be understood, however, that
- 65 the form of the apparatus and the arrangement of the parts may be varied at will without departing from the spirit and scope of the invention as defined by the appended claims.
- 70 In the drawings:
- 75 Figure 1 is an elevational view of a volumetric measuring device.
- 80 Fig. 2 is a sectional view thereof at one stage of the process.
- 85 Fig. 3 is a similar view at a later stage.
- 90 Referring to the drawings, the device selected for purposes of illustration comprises a sand bin A and an adjustable measuring hopper B. The sand bin may be suitably supported by any desired means (not shown). This bin has a circular discharge opening 1 at the bottom thereof and is provided with a gate 2 pivoted at 3 to oscillate about a vertical axis. A handle 4 on the gate serves as a means to operate the gate.
- 95 The measuring hopper B comprises an upper conical portion 5 and a lower container 6 which is generally cylindrical in form but which has inwardly sloping sides 7 at the bottom converging to define a circular discharge port 8, thereby to insure complete discharge of material from the hopper. The upper portion 5 is herein shown supported from the bin A by means of a plurality of integral brackets 9 and chains 10 which are attached at their opposite ends to the brackets and to the bin A. The container is adjustable relative to the upper portion 5 of the hopper to permit of adjustment of the volumetric content of the hopper. For this purpose the container is herein shown

suspended from the brackets 9 by means of chains 11, and adjustable screw devices 12 having hooked portions 13 are provided on each bracket to receive the free end of a chain. Should it be desired to adjust the volume of the hopper to a greater extent than that provided for by the screw devices a lower link on each chain may be caught over the hooks 13.

10 A gate 14 having a water tight gasket 14<sup>a</sup> is provided to control the discharge opening 8 of the hopper. This gate is carried on an arm 15 pivotally supported intermediate its ends at 16 on a bracket 17 which is secured 15 rigidly to the container 6. The end 18 of this arm is pivoted to an outstanding lug 19 on the gate. As herein illustrated the arm 15 is operable by means of a hand lever 20 pivoted at 21 on the bracket 17, and a toggle link 22 connecting the adjacent ends of the lever 20 and arm 15. Thus, in its closed 20 position the gate 14 is held locked by the toggle device.

23 In the apparatus illustrated in the drawings means is provided to combine water with the sand in the hopper. For this purpose a pipe 23 leading to a suitable supply of water (not shown) is connected to the lower portion of the container 6. A valve 30 24 in this pipe line is adapted to control the flow therethrough.

35 An overflow 25 is provided on the container 6 and is secured thereto by means including the bolts 26 anchored on the container. By loosening the nuts of these bolts the overflow may be raised or lowered.

40 The process consists in first measuring a predetermined volume of sand. If this volume is known in terms of apparent volume of commercial sand the hopper may be adjusted in accordance with a suitable scale (not shown) to measure this volume. If a 45 predetermined quantity of compacted sand is desired and a quantity of normally moist bulk sand is to be measured which will yield an equivalent amount of compacted sand, the volume of the measuring hopper may be set by experiment as follows:

50 A hopperful of loose moist sand is discharged into a calibrated measure and there-in compacted by tamping, rodding or other suitable methods. Should this batch of loose sand yield less than the desired volume of compacted sand, the hopper B is adjusted to measure a greater volume than before and vice versa. By a series of such experiments the volume of the hopper B is adjusted so as to measure a quantity of loose normally moist sand containing the desired volume of compacted sand.

55 With the hopper properly adjusted it is then necessary to set the overflow 25 at a level whereby the water added, combined with the moisture in the sand, gives a concrete mix of the desired consistency. A field

method well adapted for determining the proper level of the overflow, consists in making a series of experimental batches of concrete with the overflow set at different levels, until concrete of the desired consistency is obtained. Thus with the gate 14 closed, the gate 1 on the bin A is opened by operating the handle 4 whereupon sand from the bin discharges into the hopper until the hopper is full as shown in Fig. 2. By closing the 75 gate 1 the sand in the bin is cut off from the sand in the hopper, thus leaving the desired volume of loose sand in the hopper.

Water is then admitted from the supply line by opening the valve 24, until the water 80 in the hopper reaches the height of the overflow as shown in Fig. 3. This point is generally determined by allowing some water to discharge over the overflow. The valve 24 is then closed, and the experimental batch 85 of combined sand and water is used to make a batch of concrete. If the consistency of the resulting mix is other than that desired, the nuts on the bolts 26 are loosened and the overflow is raised or lowered depending upon 90 whether the concrete was too dry or wet. By a series of such experimental batches the overflow may be adjusted to a level which will provide the water necessary for the desired consistency of concrete providing the absolute volume of each batch of the premeasured loose sand does not vary. With the volume of the hopper B adjusted and the overflow 95 set at the selected level, the process consists of the following steps. First the 100 predetermined volume of normally moist sand is measured by filling the hopper from the bin A. Water is then admitted from the pipe 23 until it reaches the level of the overflow whereupon the valve is closed. The 105 mass of combined sand and water is then used in making a batch of concrete.

110 It is apparent that by this process the moisture introduced into the container as moisture in the sand, becomes a part of the total water and that the total water in the container is complementary in volume to the absolute volume of the sand. Inasmuch as the variation in absolute volume of sand measured by apparent volumes is less than the moisture variation, within the range hereinbefore mentioned, it will be apparent that the variation in total water measured by this process will be less than that encountered when water and moist sand are measured independently and later combined in a mix.

115 The process is particularly well adapted for use with apparatus of simple construction and because of its ease of operation readily lends itself to field work. When used with the apparatus described herein, and this apparatus has once been calibrated, it is merely necessary for an operator to open the gate on the sand bin and thereby 120 discharge sand into the hopper until the 125 130

sand stops flowing, then by closing the gate he strikes off the sand to the predetermined volume. The valve in the water line is then opened and water permitted to flow into the 5 hopper until some of it overflows the outlet, whereupon by closing the valve the combined sand and water is ready to be mixed with the proper proportions of cement and stone and may be discharged through the 10 gate on the hopper.

I claim as my invention:

1. A process for proportioning the total water in a concrete mix which comprises measuring a predetermined volume of normally moist sand and combining water with said measured sand until the combined sand and total water equals a second predetermined volume.
2. A process for proportioning the water 20 in a concrete mix which comprises placing a premeasured quantity of normally moist sand in a container and flowing water upwardly through the sand to a predetermined level.
- 25 3. In a process for making concrete mixtures, the step of proportioning the total water as a complementary volume to the absolute volume of premeasured normally moist bulk sand.

4. The process of making concrete mixtures which consists in measuring by apparent volume a quantity of normally moist commercial or bulk sand sufficient to equal substantially a predetermined absolute volume, and then adding water to said measured sand to produce a predetermined combined volume.

5. In concrete construction, the process of measuring the sand and water for the mix which consists in introducing moist bulk sand into a hopper having a water outlet located at a predetermined level, striking off the excess sand at a predetermined point above said water outlet, admitting water to the hopper from a point below said outlet 45 until a quantity is free to run off through the outlet, and finally discharging the combined sand and water from the hopper.

6. The process of making concrete which includes a step of combining water and a 50 quantity of bulk sand having a variable moisture content until the combined elements attain a predetermined volume as determined by the predetermined proportions of the elements to constitute the mix.

In testimony whereof, I have hereunto affixed my signature.

CHARLES S. JOHNSON.